

1

2,742,148

## MIXTURES OF ALCOHOLS AS TUBING FLUIDS FOR NON-BOILABLE CATGUT

Reginald M. Banks, Rye, N. Y., assignor to Davis & Geck, Inc., Danbury, Conn., a corporation of New York

No Drawing. Application September 14, 1953,  
Serial No. 380,081

3 Claims. (Cl. 206—63.3)

This invention relates to surgical sutures of the proteinaceous type and more particularly to the packaging, preservation and conditioning of non-boilable surgical sutures. Still more particularly this invention relates to a method of improving the strength of tubed, non-boilable catgut sutures while reducing swelling and to the composition of the liquid in which non-boilable catgut sutures are customarily packaged or tubed.

Strength, flexibility, softness and size of proteinaceous surgical sutures are important physical characteristics upon which the surgeon depends for easy and rapid manipulation during an operation and the tying of tight, secure knots. Unfortunately, these characteristics, normal to gut in the natural state, are substantially lost or destroyed at one stage in the preparation of sutures due to the necessity for thoroughly drying or dehydrating the suture before it can be heat sterilized. This is for the reason that the presence of water at sterilization temperatures rapidly reduces the strength of the suture, causes it to swell, and may even convert it completely into an incoherent, jelly-like mass. As the result of drying and after sterilization, the suture, which has shrunk in size, is hard, stiff and brittle and is in no condition to be used. This is true even when sterilization is carried out in the presence of a non-aqueous inert liquid hydrocarbon such as toluol, xylene or the like, as is sometimes done.

To preserve the sterility of sterile sutures it is customary to package them individually in sealed glass tubes together with a quantity of a liquid known in the art as tubing fluid. This may be a fluid inert to the suture such as the liquid in which the suture was sterilized, in which event the tube with the suture and the liquid inside is labeled "boilable"; or it may be a different fluid or solution which reacts with the gut of the suture to soften and flexibilize it, in which event the suture is labeled "non-boilable." As so packaged or tubed each of the above sutures has its own advantages and disadvantages. Boilable sutures have the advantage that the tube containing the suture may be boiled (heat sterilized) immediately before removal of the suture to avoid danger of contamination of the suture through inadvertent contact directly or indirectly with the outside walls of the tube during removal. A disadvantage accompanying the use of such sutures is that they must be soaked in water or other conditioning solution under aseptic conditions to soften and flexibilize them before they can be used.

Non-boilable sutures, however, are softened and flexibilized by the liquid in the tube and are available for use substantially immediately upon removal. They cannot be boiled, however, or subjected to sterilizing temperatures because of the damaging effect of the tubing

2

fluid on the suture at sterilization temperatures. This disadvantage as to non-boilability has in part been obviated by packaging the suture in two or more sealed, sterile containers, with the tube or ampule containing the suture being the innermost container.

While non-boilable sutures are much to be preferred over boilable sutures for the reason that they can be used immediately, their use has been hampered by the inability of the known tubing fluids to provide a suture having optimum strength, flexibility and softness. The exact mechanism by which the fluid or solution strengthens, softens and flexibilizes the gut is not known. The protein of which gut is composed is exceedingly complex and highly reactive and its characteristics are variously changed and modified depending upon the materials and conditions to which it is subjected.

Water alone, for instance, exerts a powerful effect on gut. Under controlled conditions as to temperatures and time water is an excellent softener and flexibilizer for gut sutures but, if allowed to remain in contact with the suture for any extended period the gut swells and continues to swell until the suture is substantially devoid of tensile strength. Absolute ethyl alcohol will soften and flexibilize gut but only to a limited degree which is not generally satisfactory. Ethyl alcohol containing from 0.5% to 10% of water is commonly used as a tubing fluid, and other alcohols, namely methyl, propyl and isopropyl, both anhydrous and admixed with varying percentages of water, have been used. Methyl alcohol is ordinarily too irritating to tissue so that its use has never been particularly popular. Propyl and isopropyl alcohols, both anhydrous and admixed with water, have been used to a limited extent because they result in substantially less swelling of the gut than is possible with mixtures of ethyl alcohol and water, but here again toxicity or irritation to tissue with which it comes in contact in a wound has prevented their general adoption. An ethyl alcohol-water solution containing 20% isopropanol and 4% water has heretofore been used as a tubing fluid, but little or no advantage has been apparent from the use of this mixture over and above the use of the usual 95% ethyl alcohol-water tubing fluid. For instance, it is stated in Patent No. 2,524,772 of October 10, 1950, to Davis, that gut sutures tubes in a fluid containing 90% isopropanol and 10% water swell only about 50% as much as they do in the 20% isopropanol, 76% ethanol, 4% water mixture described above. The patent also states that on decreasing the percentage of isopropanol in the 10% water solution to 65% isopropanol and 35% water the advantages of the isopropanol-water mixture over the 20% isopropanol, 76% ethanol and 4% water mixture disappear.

I have found that the advantage in the reduction of suture swelling derived through the use of propyl or isopropyl alcohols alone or in admixture with low concentrations of water may be substantially retained by the use of only about 65% propyl or isopropyl alcohol and 10% water in admixture with about 25% of an alcohol selected from the group consisting of methanol, ethanol and tertiary butanol. I have found that minimum swelling is obtained in the use of the above mixture when tertiary butyl alcohol is used. Compared with the standard tubing fluid consisting of 95% ethyl alcohol and 5% water, swelling of the suture is reduced in general to substantially less than one-half as shown in the following table.

## Table

| Solution                     | Size 000                    |       | Size 00                |                             | Size 0 |                        | Size 1                      |       |
|------------------------------|-----------------------------|-------|------------------------|-----------------------------|--------|------------------------|-----------------------------|-------|
|                              | After 31 days at room temp. |       | Equilib. Reached, days | After 31 days at room temp. |        | Equilib. Reached, days | After 37 days at room temp. |       |
|                              | Percent Swell.              | Flex. |                        | Percent Swell.              | Flex.  |                        | Percent Swell.              | Flex. |
| 65% isoprop. alc.-anhyd.     | 2.64                        | 8.1   | 11                     | 4.64                        | 10.5   | 7                      | 7.51                        | 13.4  |
| 25% tert.-butyl. alc.-anhyd. |                             |       |                        |                             |        |                        | 1                           | 7.0   |
| 10% distilled water          |                             |       |                        |                             |        |                        | 12.8                        | 8     |
| 65% isoprop. alc.-anhyd.     | 2.91                        | 8.0   | 7                      | 6.20                        | 10.1   | 7                      | 6.11                        | 11.9  |
| 25% ethyl. alc.-anhyd.       |                             |       |                        |                             |        |                        | 1                           | 8.11  |
| 10% distilled water          |                             |       |                        |                             |        |                        | 11.6                        | 8     |
| (control)                    | 7.58                        | 6.9   | 11                     | 12.77                       | 7.2    | 7                      | 13.8                        | 12.5  |
| 95% ethyl. alc. sda-42       |                             |       |                        |                             |        |                        | 1                           | 15.24 |
|                              |                             |       |                        |                             |        |                        | 10.0                        | 8     |

The results set forth in the table were obtained by the following procedure:

Thirty strands each of sizes 1, 0, 00 and 000 of plain catgut 3½ inches long were gauged for diameter over a portion mid-way of their lengths and the gauged area marked with two India ink spots. The smallest diameter within the area marked was recorded for each strand. Each strand was then put in a 12 mm. tube and oven dried and sterilized. After sterilization the tubes were placed in a desiccator over calcium chloride until the diameters of the strands became constant. At this time 12 tubes of each size were filled with one of the two test solutions and 12 tubes of each size were filled with the other of the two test solutions. The remaining 6 tubes of each size were filled with the control solution and all the tubes were corked with cork stoppers. The strands were then gauged at periodic intervals according to U. S. P. XIV procedures and the average percent swelling determined for each size in each of the two test solutions and in the control solution as shown in the table. The average percent flexibility of the strands as indicated in the table was determined at the end of the experiment.

In addition to the reduction in swelling of the sutures tubed in the solutions of the composition of the present invention it will be seen that this decrease in swelling is accomplished without substantial decrease in flexibility. The quantity of ethyl or tertiary butyl alcohol used also

lowers the overall toxicity of the solution. The tubing fluids of the present invention give equally improved results when used for tubing "chromic" or chrome-tanned catgut sutures, and in fact may be used to tube all types of non-boilable catgut sutures with or without needles attached, and may contain a small percentage, say .025, of phenyl-mercuric benzoate or other appropriate anti-septic if desired.

I claim:

1. As an article of manufacture, a sealed container having therein in combination a proteinaceous suture and a small quantity of a tubing fluid comprising 65% of a propyl alcohol, 10% water and 25% of tertiary butyl alcohol.
2. As an article of manufacture, a sealed container having therein in combination a proteinaceous suture and a tubing fluid comprising 65% isopropyl alcohol, 10% water and 25% tertiary butyl alcohol.
3. As an article of manufacture, a sealed container having therein in combination a proteinaceous suture and a tubing fluid comprising 65% normal propyl alcohol, 10% water and 25% tertiary butyl alcohol.

40

## References Cited in the file of this patent

## UNITED STATES PATENTS

- 2,524,772 Davis Oct. 10, 1950  
2,694,487 Powers Nov. 16, 1954

45